

Patented Dec. 22, 1925.

1,566,310

# UNITED STATES PATENT OFFICE.

ALBERT L. CLAPP, OF DANVERS, MASSACHUSETTS, ASSIGNOR TO BECKWITH MANUFACTURING COMPANY, OF BOSTON, MASSACHUSETTS, A CORPORATION OF MASSACHUSETTS.

## FIBER BOARD.

No Drawing.

Application filed August 23, 1921. Serial No. 494,638.

To all whom it may concern:

Be it known that I, ALBERT L. CLAPP, a citizen of the United States, residing at Danvers, in the county of Essex and State of Massachusetts, have invented new and useful Improvements in Fiber Board, of which the following is a specification.

This invention relates to the manufacture of hard, dense, fiber board or like products. I have discovered that, if cellulose fibers are beaten for a sufficient period of time to ensure the hydration thereof and are then formed by suitable paper-making machinery into a sheet of the desired thickness, it is possible by heat and pressure to convert the sheet or portions thereof into a relatively hard, dense, and more or less horny product.

For example, if sulphate pulp or waste kraft paper with sufficient water to insure circulation be beaten hard in a beating engine for 20 to 24 hours, the fibers are highly hydrated, and the stock is "slow" or slimy due to the mucilaginous hydrate thereby produced while the "felting" property of the fibers is not destroyed. Such stock may then be formed into a sheet of the desired thickness by a "wet machine" so-called, removed from the make-up roll and dried. Button blanks may then be die-cut or stamped from the sheet, and, when such blanks are then subjected in a suitable mold to a pressure of about 2500 pounds per square inch while heated to a temperature of 160° to 220° F., the buttons thereby produced are

hard, dense and horny, due to the cementing or binding action of the hydrated fibers. With less beneficial results, the stock may be beaten for 8 to 10 hours, whereas, when beaten for less than 5 or 6 hours, the fibers of the sheet thereafter produced have no binding or cementing action when subjected to heat and pressure. Apparently the gelatinous or mucilaginous hydrate produced by the long beating of the cellulose stock, even when the uncombined water is removed during the drying of the sheet, is effective, when the material is subjected to heat and high pressure, in cementing the mass together.

For increasing the water-resistant qualities of the molded or compressed product, I may add to the stock a quantity of sodium resinate, say 5% to 10% by weight of the dry cellulose stock; and, when the beating operation has been carried on to the desired extent, aluminum resinate may be precipitated

by the addition of an equal amount of alum to the stock.

In lieu of the specific cellulosic raw material hereinbefore referred to, I may use any other suitable cellulosic material such as 60 mechanical or chemical wood pulp, rags, rope, waste paper, etc.

A dense board as thus produced may be employed as a base for phonograph records, printing plates and the like. In addition, it 65 may be used for electric insulation and for other uses to which "hard fiber" has heretofore been employed.

For use as printing plates, the compressed board may be coated or not as desired. Under heat and high pressure it receives and retains the impressions of a matrix. The cellulose-mucilage under heat and pressure cements and binds the fibrous mass into a homogeneous horn-like, dense, hard article, 75 whether the latter be a sheet, a plate, a phonograph record, a button or other element.

If it be desired to impart a luster or fine finish to the finished product, as in the case 80 of buttons for example, the blanks may be coated with a solution of gums, resins, or phenol resins, and, after the solvent has evaporated, the blanks are subjected to heat and high pressure in suitable molds. Buttons thus formed have a fine appearance and polish or luster.

What I claim is:—

1. The herein described method of making dense hard fiber board, which comprises 90 beating cellulosic material until the fibers are well hydrated, then sheeting the stock on a paper-making machine and drying the same, and subjecting the sheet or portions thereof to heat and high pressure of an 95 order of about 2500 pounds to the square inch.

2. The herein described method of making dense hard fiber board, which comprises 100 beating cellulosic material until the fibers are well hydrated, then sheeting the stock on a paper-making machine and drying the same, cutting blanks from such sheet, coating such blanks with a resinous solution, and molding such blanks under heat and 105 high pressure.

In testimony whereof I have affixed my signature.

ALBERT L. CLAPP.